

1

3,671,184

## MODIFYING CELLULOSIC FABRIC WITH DICARBOXYLIC ACIDS TO IMPART WATER-DISPERSIBILITY

John Anthony Cuculo, Raleigh, N.C., assignor to E. I. du Pont de Nemours and Company, Wilmington, Del.  
No Drawing. Filed May 26, 1969, Ser. No. 827,975  
Int. Cl. D06m 13/20; A61f 13/16

U.S. Cl. 8—120

4 Claims

### ABSTRACT OF THE DISCLOSURE

Cellulose half-acid esters are prepared by impregnating cellulosic material with a concentrated aqueous solution of an organic dicarboxylic acid anhydride and ammonia, heating the impregnated cellulose material at 160° to 210° C. for about 10 to 60 seconds until the desired ester substitution has occurred, washing the esterified cellulose, and neutralizing the free carboxyl radicals with a solution containing metal ions. The examples illustrate the effect of varying the temperature and time on the degree of substitution obtained with succinic, phthalic and maleic anhydrides. Cellulosic fibers can be modified so that fabrics will disperse readily in water.

### FIELD OF INVENTION

This invention relates to a process for reacting organic dicarboxylic acid anhydrides with cellulosic materials, and is more particularly concerned with modifying cellulosic fibers of fabric materials to make them dispersible in merely turbulent water, i.e., without the use of high energy equipment such as paper beaters or paper mills.

When diapers, or fabrics used for other sanitary purposes, are to be disposed of without washing for reuse, it is desirable that they be dispersible in water so that they can be flushed away as sewage. This can be accomplished by chemical modification of fibers to make the surfaces slippery when wet. Fabrics composed of such fibers will come apart when agitated in water, and the dispersed fibers can be flushed away without clogging sewage systems. The present invention provides an economical process for substituting suitable hydrophilic radicals on the surface of cellulosic fibers. The degree of substitution can be controlled so that fabrics of the modified fibers will have adequate strength when dry or wet with salt solutions, but will be dispersible in turbulent city water.

### SUMMARY OF THE INVENTION

In the process of the present invention, cellulosic material is reacted with a substantially saturated aqueous solution of a partial ammonium salt of an organic dicarboxylic acid by heating within the temperature range of 160° to 210° C. to form a reaction product weighing, after washing to remove excess reactants and drying, about 10% to 40% more than the original dry cellulosic material. It is believed that the dicarboxylic acid has reacted with cellulose hydroxyl groups to form half esters of the dicarboxylic acid. The extent of reaction with cellulose hydroxyl groups may be stated in terms of the degree of substitution (D.S.) which is the ratio of the moles of acid esterified to the moles of  $C_6H_{10}O_5$  in the cellulosic material, the maximum D.S. being 3.0. When modifying cellulosic fibers to make fabrics of them dispersible, the reaction is preferably conducted so as to provide a D.S. of about 0.15 to about 0.40.

A preferred treatment for fabrics of cellulosic fibers is to dissolve an organic dicarboxylic acid anhydride in water containing sufficient ammonium hydroxide to provide 1 to about 1.5 moles of ammonia per mole of an-

2

hydride, impregnate the fabric with sufficient solution to provide 1.5 to 20 times the amount of acid to be reacted with the cellulose, heat the fabric within the temperature range of 160° to 210° C. until the cellulosic fibers have a D.S. of about 0.15 to about 0.40, wash the fabric to remove excess reactants, and neutralize the free carboxylic acid groups with a buffered alkaline solution containing deswelling salt to form the sodium salt of the acid groups.

The fabric may be soaked in a substantially saturated solution of the organic dicarboxylic acid anhydride and ammonium hydroxide until the fabric picks up about 1 to 3 times its weight of the solution. The solution may contain a minor amount of esterification catalyst. Alternatively, the fabric may be wet with ammonium hydroxide solution and then passed through molten acid anhydride to form a saturated solution in the fabric.

### DETAILED DESCRIPTION

#### Reactants

Preferred dicarboxylic acids include succinic acid, maleic and ortho-phthalic acid as well as substitution products containing such groups as alkyl, alkoxy, halogen, nitro, and hydroxyl. Suitable acids include itaconic acid, citraconic acid, and hydroxy ortho-phthalic acids.

The cellulosic material can be in any convenient form such as fibers, woven or knitted fabrics of the fibers, non-woven fabrics, wood pulp, cotton linters, films, granules, or powders. Regenerated cellulose in the form of fibers is preferred. This includes all cellulose fibers formed from a solution such as viscose rayon, cuprammonium rayon, deacetylated cellulose acetate fibers, denitrated nitro-silk and the like. Fibers made from low-substituted cellulose derivatives such as hydroxy ethyl cellulose or methyl cellulose may also be used.

#### Reaction considerations

The following discussion of process and examples will be in terms of cellulosic fibers, and more frequently fabrics of the fibers, although it will be understood that the comments also apply to other cellulosic materials, as powders, films, etc. Near-saturated solutions are preferred in order to keep the amount of water to be dried out to a minimum. Unless otherwise specified, all solution concentrations are expressed as percent by weight.

The reactant solution is conveniently prepared by mixing water and ammonium hydroxide and then dissolving the acid anhydride. The heat of solution and reaction will assist in dissolving the acid anhydride to the extent desired. External heat can be applied to keep the solution in solution. Temperatures of about 60° C. are useful for acid anhydrides as succinic and maleic. Phthalic anhydrides require a higher temperature of about 80–85° C. to obtain the concentration required. Catalyst, if used, can be added after the anhydride is dissolved.

The reaction with some anhydrides proceeds at a satisfactory rate merely as the result of the application of heat and no catalyst is necessary. However, catalysts may be used if desired. Materials that have an effect in promoting the esterification include sulfamic acid, p-toluenesulfonic acid, zinc chloride, magnesium chloride, and the like.

When using a solution, fabric is soaked in the acid anhydride solution long enough to thoroughly wet it so it will retain the quantity of reagent desired. The term "pick-up" (i.e., weight of solution in the fabric/original dry weight of fabric) is used to indicate the amount of reagent applied. The pick-up desired will vary with the particular acid used, the concentration of the acid, and the extent of reaction. In general, the fabric should contain from 1.5 to 20 or more times the theoretical amount

of acid for the extent of reaction desired. Pick-ups of from about 1 to 3 are conveniently used.

Excess solution picked up in the soaking process is removed by centrifuging or by the application of pressure. In the preferred continuous process, using a warp sheet or pre-formed fabric, the fibers are run through a dip tank of solution, and then between conventional squeeze rolls adjusted to leave the desired amount of liquid on the fibers. Alternatively, the exact amount of solution needed is applied directly to the moving warp sheet or fabric by means of a conventional padder. In this case no excess solution need be removed.

The fibers that have been treated with the required amount of acid reagent solution may be dried slowly at room temperature or slightly elevated temperature. In the interest of speed and economy it is preferred to dry the fibers as part of the high-temperature reaction operation while maintaining a high humidity atmosphere during the drying stage of the process.

The heating of the fibers to bring about reaction can be carried out by any known means that allows reasonably careful control of the time and temperature of reaction. Hot circulating air ovens, or, in the case where sheet materials are used, heated rolls may be used. In the preferred process, using a pre-formed entangled-fiber non-woven fabric, a tenter frame provides a convenient means for holding the fabric flat and at the desired dimensions while exposing it to a controlled flow of hot air to drive off water and bring about the esterification reaction.

The process can also be carried out by passing a fabric wet with ammonium hydroxide solution through a bath of molten acid anhydride and then heating. This is especially useful with the lower melting anhydrides such as maleic.

#### Purification and after treatments

The fibers or fabric obtained at the end of the high-temperature reaction are contaminated with excess acid anhydride, small amounts of the corresponding dibasic acid, and traces of various decomposition products. These impurities are easily removed by means of a water wash. Since the half ester formed in the reaction is in the free acid form, or ammonium salt form to a small extent, the fibers of the more preferred products (D.S. of 0.2 to 0.3) are low-swelling and no damage is sustained by the fibers or fabric in this treatment.

The final washed fabric, whether arrived at by modifying pre-formed fabric or by forming fabric from pre-modified fibers, is next converted to the more useful high-swelling form by treatment with a base, preferably a slightly alkaline buffer such as disodium phosphate to form the sodium salt of the acid groups. In order to prevent excessive swelling and possible solution or other damage in the alkaline medium the buffer may be mixed with a solution of a deswelling salt such as sodium sulfate. Other strongly ionizing salts such as ammonium sulfate or sodium citrate may also be used, but sodium sulfate appears to be the most effective and economical, and the most desirable as a minor residual solid in the final fabric. Suitable salts are discussed in U.S. Pat. No. 3,328,892 to Man dated July 4, 1967. In order to prevent stiffening or harshening during drying, the fabric is dried directly while still wet with the deswelling buffered salt solution. Mechanical working during drying helps to soften the fabric and remove excess free salt. If a salt-free final product is desired, it may be obtained in a softened form by extracting the buffered salt solution with aqueous alcohol or acetone, rinsing in dry alcohol or acetone, and then drying with heat. Alternatively, the use of salt may be minimized by neutralizing the free acid groups in the fabric with an aqueous alcohol solution of a buffer or dilute alkali, followed by an alcohol or acetone wash, and then drying with heat.

The following neutralization baths are used in the examples:

| Bath   | Percent                         |                                  |        |     |
|--------|---------------------------------|----------------------------------|--------|-----|
|        | Na <sub>2</sub> SO <sub>4</sub> | Na <sub>2</sub> HOP <sub>4</sub> | Bleach | pH  |
| A----- | 8.5                             | 1.5                              | 0.75   | 8.5 |
| B----- | 8.5                             | 1.5                              | 0.75   | 8.0 |
| C----- | 4.0                             | 2.0                              | 0.75   | 8.5 |
| D----- | 4.0                             | 2.0                              | 0.0    | 8.5 |
| E----- | 8.5                             | 1.5                              | 0.0    | 8.0 |
| F----- | 4.0                             | 2.0                              | 0.75   | 8.0 |

The ingredients are dissolved in water and the pH adjusted to the noted value by the addition of dilute base. The "bleach" is commercial sodium hypochlorite solution. Other agents can be added as desired.

#### Utility of the products

In addition to the preferred utility already discussed, the products of the process are also useful in a number of other ways. They may be used as cation exchange mediums. The sodium or ammonium salt forms are soluble in dilute alkali and the solutions are useful in the formation of films and fibers. Fibers of the products may be treated with heavy metal ions such as copper ions to give increased resistance to mildew and decay. The moisture absorbency and dyeability of cellulosic materials such as cotton or rayon can be increased by modifying the fibers in accordance with this process.

#### Preparation of nonwoven fabric (A)

Nonwoven fabrics of entangled fibers are conveniently made by treating a fibrous web with fine, closely-spaced, liquid streams issuing from orifices at high pressures as taught by British Pat. No. 1,088,376, published Oct. 25, 1967.

Typically a web of 1.0 ounce per square yard (34 grams per square meter or g./m.<sup>2</sup>) of 1.5 denier per filament (d.p.f.), 0.75 inch (1.9 cm.) long rayon staple, in a random array made by air deposition, is placed on a 24 x 24 mesh per inch (per 2.54 cm.) screen (16% open area) and passed at 6 yds./minute (5.5 m.p.m.) under 3 rows of water streams coming from orifices having an upper cylindrical section of 0.005 inch (0.13 mm.) diameter with a lower frustoconical section as an exit and spaced 40 per inch (per 2.54 cm.) at pressures of 400, 500 and 600 pounds per square inch (28, 35 and 42 kilograms per square centimeter, kg./cm.<sup>2</sup>), respectively, (all pressures are gauge). The orifices are about 12 mm. above the web. This strong, integral nonwoven fabric (A) having a pattern of apertures is used in the examples. The fabric has a strip tensile strength of 3.3 lb./in. (590 g./cm.) when dry, a wet coefficient of friction of 1.32 and when tested as defined below, substantially zero dispersibility and about 0.7-0.9 single layer absorbency.

#### TEST METHODS

##### Dispersibility

The dispersibility is determined in a 250 ml. filter flask having an added side arm at the bottom of the conical wall and containing a magnetically rotated bar. The bar is 3.8 cm. long by 8 mm. in diameter, weighs 11.73 grams and is rotated at 500 revolutions per minute. A 3 x 3-inch sample of fabric is folded in half and inserted under the surface of the water (at the top side arm). Tap water at about 25° C. is added through the bottom tube at a rate of 0.70 liters/minute for a period of 2 minutes. The effluent liquid from the upper side arm is filtered and the residue dried to constant weight at 100° C. to give the weight of fibers dispersed. The contents of the filter flask are filtered after the test and dried to yield the weight of undispersed fibers. The percent dispersibility is equal to 100 times the weight of fibers dispersed divided by the total weight of fibers recovered. Conventional toilet tissues have a dispersibility of 7% in this test.

In addition to the above quantitative result, the notes under dispersibility also include a visual estimate of the percent of fabric that has dispersed in 2 minutes or the

## 5

time (less than 2 minutes) when the fabric has completely dispersed.

Nonwoven fabrics processed by this invention having a weighed dispersibility of from 20% to about 100% or a visual dispersibility from about 80% to about 100% are flushable in normal household toilets in the form of diapers. Those fabrics having dispersibilities as low as 4% (by weight) or 10% (visual) may be dispersed in water with relatively mild agitation.

The degree of substitution of a cellulose product of this invention is calculated from carboxyl group analysis. A portion of a sample is treated with sulfuric acid to insure conversion to the carboxylic acid form, washed free of acid, and then dried. A weighed portion of the dried product is shaken with a measured amount of calcium acetate solution. The acetic acid liberated is back titrated with 0.1 N NaOH and the percent of acid groups is calculated.

## Single layer absorbency

The single layer (designated SL) absorbency method has been devised to measure fiber absorbency in the fabric state and to minimize interstitial water. A 3 in. x 3 in. (7.6 x 7.6 cm.) sample in a 100-mesh screen basket is immersed for 1 minute in 150 ml. of a 0.1% aqueous NaCl solution and the basket is then dipped in and out of the solution 5 times and drained for 15 seconds. The procedure is repeated in a fresh salt solution and the sample soaked for 5 minutes before draining the basket for 30 seconds. The wet sample is dropped from the basket onto a dry blotter and immediately dropped from the first blotter to a second dry blotter and covered with another dry blotter. The 2 blotters (5 x 5 in.) and intermediate sample are covered with a 5 in. x 5 in. aluminum plate and a weight added on top to give a total weight for the weight and plate of 3 kg. The sample is pressed at the 3 kg. pressure for 5 minutes and weighed immediately. The sample is dried for 2 hours in a hot air oven at 125° C., cooled in a desiccator and weighed immediately. The SL absorption is obtained by dividing (pressed wet weight minus dry weight) by the dry (final) weight to yield grams of solution/grams of dry fabric.

If the SL absorbency is less than 1.0 g./g., the determination should be repeated using blotters that have been slightly dampened (about 0.2 g./g. of dry blotter) with a fine spray of the salt solution. Such a procedure avoids a false reading caused by some of the solution from the fibers (as well as interstitial) being absorbed by the dry blotters.

Conversely, if the blotters appear to be fully soaked, the procedure should be repeated with the addition of a paper towel on the outside face of each blotter as all of the interstitial solution is not removed otherwise.

Strip tensile strength and elongations are measured on an Instron testing machine using a 2-inch (5.0 cm.) length between jaws of a 1.0 inch (2.54 cm.) wide sample and elongating at 50% per minute. For wet tensile strengths, samples are soaked in the appropriate liquid for 5 minutes at room temperature and then clamped in the tester and broken in air.

## EXAMPLE I

This example illustrates a continuous process for the chemical modification of a rayon nonwoven fabric.

The nonwoven rayon fabric (A) described previously, is passed through a tank containing a solution at about 60° C. of 40% succinic anhydride and the stoichiometric amount of ammonia (from NH<sub>4</sub>OH) needed for the monoammonium salt. The fabric is squeezed by a pair of rubber-covered rolls to a pick-up of 1.7. The wet fabric is continuously passed through a commercial fabric oven (Benz) where it is exposed to opposed jets of air at 205° C. for a period of about 57 seconds to give brown colored fabrics. The baked fabric is washed with tap water and then neutralized and bleached (to an off-white

## 6

color) in neutralization bath F and air dried. The properties of the product are as follows:

## Strip tensile strength:

Dry lb./in.: 4.5  
(G./cm.): (800.)  
In tap water lb./in.: 0.02  
(G./cm.): (3.6)  
In 1% NaCl lb./in.: 0.07  
(G./cm.): (12.5)

## Dispersibility:

Percent fibers recovered: 35.

Percent fabric dispersed: 100% in 7 seconds

Coefficient of friction, wet: 0.52  
SL absorbency (g. sol./g. fabric): 3.01  
D.S.: 0.26

Diapers are assembled with a layer of the product, wood fluff, crepe tissue wadding, wood fluff and the product in order. The outer layers of the product fabric are 11 x 14 inch (28 x 35 cm.) and the inner core of wood fluff and crepe tissue are 5 x 12 inch (12.7 x 30 cm.). The two fabric layers are glued together around the edges of the core with about 3 mm. spots of a water-soluble adhesive spaced about 5 cm. apart. The diapers can be flushed in a home-type toilet with tap water (200 p.p.m. hardness) after 3 to 5 dips without causing the toilet-bowl to overflow or lodging on wire hooks located in the exit pipe of the toilet.

Repetition of the above process using a pick-up of 1.6 gives a modified fabric with a dispersibility of 14%.

## EXAMPLE 2

This example shows the effect of the concentration of succinic anhydride solutions on the process.

Solutions are prepared by mixing water with ammonium hydroxide (1 mole of NH<sub>3</sub>/mole of anhydride) and then adding the succinic anhydride slowly. No external heat is required to effect complete solution but the solutions are heated to maintain them at about 50° C. while using.

Preweighed, 5 x 8-inch (12.7 x 20 cm.) portions of the entangled rayon nonwoven fabric are immersed in the reactant solution for about 1 minute, removed and squeezed and/or pressed on blotters to a pick-up of 1.9 (i.e., 1.9 grams of solution/gram of original dry fabric). The wet fabric is clipped between 2 "Teflon®" screens which are then hung in a stainless steel box with slots on the top and bottom in a circulating air oven adjusted to 205° C. A thermocouple is in contact with the fabric.

After heating for 90 seconds, the fabric is removed washed with water, neutralized in bath E, blotted and air dried.

Results are given in Table I as items (a)-(e).

The as-baked products are strong both dry and wet and have a tan color.

The extent of reaction as judged by the dispersibility values increases with the concentration of the anhydride in the reactant solution.

## EXAMPLE 3

This example shows the effect of an esterification catalyst on the reaction with succinic anhydride.

Preweighed 5.5 x 5.5 inch (14 x 14 cm.) portions of the entangled rayon nonwoven fabric are treated with an aqueous solution containing 50% succinic anhydride and 1 mole of NH<sub>3</sub>/mole of anhydride to a pick-up of 1.9 (item (f)).

The wet fabrics are clipped to a stainless-steel screen and hung in a tube oven so that hot air enters the oven through a diffusing plate, passes through the fabric and exits from the oven. A thermocouple is in contact with the fabric. The oven temperature (205° C.) is measured by a thermocouple downstream of the fabric.

The procedure is repeated with the addition of sulfamic acid (2% of the weight of succinic anhydride) to the solution to make item (g).

The baked fabrics are washed in water, neutralized and bleached in bath A, blotted and air dried. Results are given in Table I as items (f) and (g). The as-baked fabrics are strong; Item (f) has a rather brown color and item (g) an off-white color; both are bleached to a satisfactory white.

The increased extent of reaction using the catalyst is obvious from the dispersibility values of the products.

#### EXAMPLE 4

This example shows the effect of time on the reaction between rayon and succinic anhydride.

The procedure of item (g) of Example 3 is repeated with reaction times of 10 to 60 seconds to give items (h)–(m) as reported in Table I. The color of the as-baked fabrics increases with the reaction time from an

15

sion of the sulfamic acid. After baking for 60 seconds it is washed and neutralized in bath A.

All items are strong in the as-baked state except (f). It is speculated that the lower tensile of item (f) is due to an increased degradation of the rayon. The color of the as-baked items increases with reaction time from an off-white to brown. All are bleached in the neutralization bath.

#### EXAMPLE 6

This example shows the effect of temperature with small variations in time on the reaction between rayon and phthalic anhydride.

The procedure of Example 5 using sulfamic acid as a catalyst is followed with oven temperatures and times as given in Table II for items (g)–(m) and using neutralization bath C. The solution for item (m) contains 36.6% phthalic anhydride.

All as-baked fabrics are strong wet and dry and colored from tan to brown. All are bleached in the neutralization bath.

TABLE II

| Item             | Reaction time, seconds | Temperature, °C. |                   |                     | Dispersibility  |                         |       | S.I. absorbency |
|------------------|------------------------|------------------|-------------------|---------------------|-----------------|-------------------------|-------|-----------------|
|                  |                        | Oven             | Maximum on fabric | Neutralization bath | Fibers, percent | Visual, percent/seconds | D.S.  |                 |
| a <sup>1</sup> — | 60                     | 205              | 202               | A                   | 5               | 15/120                  | ----- | -----           |
| b <sup>1</sup> — | 10                     | 205              | 164               | B                   | 4               | 15/120                  | 0.15  | -----           |
| c <sup>1</sup> — | 20                     | 205              | 194               | B                   | 13              | 75/120                  | 0.20  | -----           |
| d <sup>1</sup> — | 30                     | 205              | 200–202           | B                   | 35              | 90/120                  | 0.22  | -----           |
| e <sup>1</sup> — | 40                     | 205              | 204               | B                   | 36              | 85/120                  | 0.21  | -----           |
| f <sup>1</sup> — | 50                     | 205              | 206               | B                   | 65              | 100/4                   | 0.23  | -----           |
| g <sup>1</sup> — | 50                     | 190              | 184               | C                   | 5               | 10/120                  | ----- | -----           |
| h <sup>1</sup> — | 50                     | 195              | 190               | C                   | 5               | 50/120                  | ----- | -----           |
| i <sup>1</sup> — | 50                     | 200              | 193               | C                   | 10              | 70/120                  | ----- | -----           |
| j <sup>1</sup> — | 40                     | 200              | 185               | C                   | 4               | 50/120                  | ----- | -----           |
| k <sup>2</sup> — | 50                     | 205              | 201               | C                   | 46              | 95/40                   | .18   | -----           |
| l <sup>2</sup> — | 40                     | 205              | 201               | C                   | 22              | 90/120                  | .18   | 1.94            |
| m <sup>2</sup> — | 30                     | 205              | 196–201           | C                   | 42              | 100/20                  | ----- | -----           |

<sup>1</sup> No catalyst.

<sup>2</sup> Pick-up 1.8.

NOTE.—Reactant solution 36.3% phthalic anhydride, 1.5 moles NH<sub>3</sub>/mole of anhydride and 2% (based on anhydride) of sulfamic acid as a catalyst; pick-up 1.9.

off-white for item (h) to a dark brown for item (m). All are satisfactorily bleached in the neutralization bath.

Item (m) has a tensile strength in distilled water of 0.025/0.015 (MD/XD) lb./in. (4.5/2.7 g./cm.) and a

TABLE I

| Item | Reactant solution  |                               | Reaction time, seconds | Temperature, °C., maximum on fabric | Neutralization bath | Dispersibility  |                         |       | D.S.  |
|------|--------------------|-------------------------------|------------------------|-------------------------------------|---------------------|-----------------|-------------------------|-------|-------|
|      | Anhydride, percent | Percent <sup>1</sup> catalyst |                        |                                     |                     | Fibers, percent | Visual, percent/seconds | D.S.  |       |
| a—   | 20                 | 0                             | 90                     | 192                                 | E                   | 5               | <15/120                 | ----- | ----- |
| b—   | 25                 | 0                             | 90                     | 195                                 | E                   | 12              | 25/120                  | ----- | ----- |
| c—   | 30                 | 0                             | 90                     | 191                                 | E                   | 33              | ~90/120                 | ----- | ----- |
| d—   | 40                 | 0                             | 90                     | 186                                 | E                   | 41              | ~90/120                 | ----- | ----- |
| e—   | 50                 | 0                             | 90                     | 190                                 | E                   | 69              | 100/7                   | ----- | ----- |
| f—   | 50                 | 0                             | 60                     | 200                                 | A                   | 15              | ~50/120                 | ----- | ----- |
| g—   | 50                 | 2                             | 60                     | 202                                 | A                   | 55              | 100/10                  | ----- | ----- |
| h—   | 50                 | 2                             | 10                     | 158                                 | A                   | 2               | <10/120                 | 0.073 | ----- |
| i—   | 50                 | 2                             | 20                     | 192                                 | A                   | 5               | ~10/120                 | 0.17  | ----- |
| j—   | 50                 | 2                             | 30                     | 198                                 | A                   | 19              | 45/120                  | 0.26  | ----- |
| k—   | 50                 | 2                             | 40                     | 192                                 | A                   | 38              | 100/10                  | 0.28  | ----- |
| l—   | 50                 | 2                             | 50                     | 204                                 | A                   | 38              | 100/7                   | 0.31  | ----- |
| m—   | 50                 | 2                             | 60                     | 204                                 | A                   | 32              | 100/5                   | 0.30  | ----- |

<sup>1</sup> Percent (based on anhydride) of sulfamic acid.

NOTE.—205° C. oven used for all items; reactant solution contains 1 mole NH<sub>3</sub>/mole of anhydride; pick-up 1.9 for all.

#### EXAMPLE 5

This example shows the effect of reaction time on the reaction between phthalic anhydride and rayon.

A solution is made by dissolving 36.3% orthophthalic anhydride in a mixture of water and ammonium hydroxide that gives 1.5 moles NH<sub>3</sub>/mole of anhydride. Sulfamic acid (2% of the weight of the anhydride) is added. The extra 0.5 mole of NH<sub>3</sub> is used to help dissolve the anhydride. The solutions are kept at about 80°–90° C. to maintain complete solution.

Fabrics are treated with the solution to a pick-up of 1.9 and baked in the oven of Example 3 at 205° C. for different times of from 10 to 60 seconds. The baked fabrics are washed in water, neutralized in bath B, blotted and air dried to give items (b)–(f) of Table II.

Item (a) of Table II is made as above with the omis-

60  
70  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
330  
331  
332  
333  
334  
335  
336  
337  
338  
339  
340  
341  
342  
343  
344  
345  
346  
347  
348  
349  
340  
341  
342  
343  
344  
345  
346  
347  
348  
349  
350  
351  
352  
353  
354  
355  
356  
357  
358  
359  
350  
351  
352  
353  
354  
355  
356  
357  
358  
359  
360  
361  
362  
363  
364  
365  
366  
367  
368  
369  
360  
361  
362  
363  
364  
365  
366  
367  
368  
369  
370  
371  
372  
373  
374  
375  
376  
377  
378  
379  
370  
371  
372  
373  
374  
375  
376  
377  
378  
379  
380  
381  
382  
383  
384  
385  
386  
387  
388  
389  
380  
381  
382  
383  
384  
385  
386  
387  
388  
389  
390  
391  
392  
393  
394  
395  
396  
397  
398  
399  
390  
391  
392  
393  
394  
395  
396  
397  
398  
399  
400  
401  
402  
403  
404  
405  
406  
407  
408  
409  
400  
401  
402  
403  
404  
405  
406  
407  
408  
409  
410  
411  
412  
413  
414  
415  
416  
417  
418  
419  
410  
411  
412  
413  
414  
415  
416  
417  
418  
419  
420  
421  
422  
423  
424  
425  
426  
427  
428  
429  
420  
421  
422  
423  
424  
425  
426  
427  
428  
429  
430  
431  
432  
433  
434  
435  
436  
437  
438  
439  
430  
431  
432  
433  
434  
435  
436  
437  
438  
439  
440  
441  
442  
443  
444  
445  
446  
447  
448  
449  
440  
441  
442  
443  
444  
445  
446  
447  
448  
449  
450  
451  
452  
453  
454  
455  
456  
457  
458  
459  
450  
451  
452  
453  
454  
455  
456  
457  
458  
459  
460  
461  
462  
463  
464  
465  
466  
467  
468  
469  
460  
461  
462  
463  
464  
465  
466  
467  
468  
469  
470  
471  
472  
473  
474  
475  
476  
477  
478  
479  
470  
471  
472  
473  
474  
475  
476  
477  
478  
479  
480  
481  
482  
483  
484  
485  
486  
487  
488  
489  
480  
481  
482  
483  
484  
485  
486  
487  
488  
489  
490  
491  
492  
493  
494  
495  
496  
497  
498  
499  
490  
491  
492  
493  
494  
495  
496  
497  
498  
499  
500  
501  
502  
503  
504  
505  
506  
507  
508  
509  
500  
501  
502  
503  
504  
505  
506  
507  
508  
509  
510  
511  
512  
513  
514  
515  
516  
517  
518  
519  
510  
511  
512  
513  
514  
515  
516  
517  
518  
519  
520  
521  
522  
523  
524  
525  
526  
527  
528  
529  
520  
521  
522  
523  
524  
525  
526  
527  
528  
529  
530  
531  
532  
533  
534  
535  
536  
537  
538  
539  
530  
531  
532  
533  
534  
535  
536  
537  
538  
539  
540  
541  
542  
543  
544  
545  
546  
547  
548  
549  
540  
541  
542  
543  
544  
545  
546  
547  
548  
549  
550  
551  
552  
553  
554  
555  
556  
557  
558  
559  
550  
551  
552  
553  
554  
555  
556  
557  
558  
559  
560  
561  
562  
563  
564  
565  
566  
567  
568  
569  
560  
561  
562  
563  
564  
565  
566  
567  
568  
569  
570  
571  
572  
573  
574  
575  
576  
577  
578  
579  
570  
571  
572  
573  
574  
575  
576  
577  
578  
579  
580  
581  
582  
583  
584  
585  
586  
587  
588  
589  
580  
581  
582  
583  
584  
585  
586  
587  
588  
589  
590  
591  
592  
593  
594  
595  
596  
597  
598  
599  
590  
591  
592  
593  
594  
595  
596  
597  
598  
599  
600  
601  
602  
603  
604  
605  
606  
607  
608  
609  
600  
601  
602  
603  
604  
605  
606  
607  
608  
609  
610  
611  
612  
613  
614  
615  
616  
617  
618  
619  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
620  
621  
622  
623  
624  
625  
626  
627  
628  
629  
630  
631  
632  
633  
634  
635  
636  
637  
638  
639  
630  
631  
632  
633  
634  
635  
636  
637  
638  
639  
640  
641  
642  
643  
644  
645  
646  
647  
648  
649  
640  
641  
642  
643  
644  
645  
646  
647  
648  
649  
650  
651  
652  
653  
654  
655  
656  
657  
658  
659  
650  
651  
652  
653  
654  
655  
656  
657  
658  
659  
660  
661  
662  
663  
664  
665  
666  
667  
668  
669  
660  
661  
662  
663  
664  
665  
666  
667  
668  
669  
670  
671  
672  
673  
674  
675  
676  
677  
678  
679  
670  
671  
672  
673  
674  
675  
676  
677  
678  
679  
680  
681  
682  
683  
684  
685  
686  
687  
688  
689  
680  
681  
682  
683  
684  
685  
686  
687  
688  
689  
690  
691  
692  
693  
694  
695  
696  
697  
698  
699  
690  
691  
692  
693  
694  
695  
696  
697  
698  
699  
700  
701  
702  
703  
704  
705  
706  
707  
708  
709  
700  
701  
702  
703  
704  
705  
706  
707  
708  
709  
710  
711  
712  
713  
714  
715  
716  
717  
718  
719  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
720  
721  
722  
723  
724  
725  
726  
727  
728  
729  
730  
731  
732  
733  
734  
735  
736  
737  
738  
739  
730  
731  
732  
733  
734  
735  
736  
737  
738  
739  
740  
741  
742  
743  
744  
745  
746  
747  
748  
749  
740  
741  
742  
743  
744  
745  
746  
747  
748  
749  
750  
751  
752  
753  
754  
755  
756  
757  
758  
759  
750  
751  
752  
753  
754  
755  
756  
757  
758  
759  
760  
761  
762  
763  
764  
765  
766  
767  
768  
769  
760  
761  
762  
763  
764  
765  
766  
767  
768  
769  
770  
771  
772  
773  
774  
775  
776  
777  
778  
779  
770  
771  
772  
773  
774  
775  
776  
777  
778  
779  
780  
781  
782  
783  
784  
785  
786  
787  
788  
789  
780  
781  
782  
783  
784  
785  
786  
787  
788  
789  
790  
791  
792  
793  
794  
795  
796  
797  
798  
799  
790  
791  
792  
793  
794  
795  
796  
797  
798  
799  
800  
801  
802  
803  
804  
805  
806  
807  
808  
809  
800  
801  
802  
803  
804  
805  
806  
807  
808  
809  
810  
811  
812  
813  
814  
815  
816  
817  
818  
819  
810  
811  
812  
813  
814  
815  
816  
817  
818  
819  
820  
821  
822  
823  
824  
825  
826  
827  
828  
829  
820  
821  
822  
823  
82

Item (a) is made without sulfamic acid in the reactant solution.

All products are strong in the as-baked state, wet and dry, and are colored from off-white or yellow to light tan 5 before bleaching.

TABLE III

| Item               | Reaction time, seconds | Temperature, ° C. |                   | Neutralization bath | Dispersibility  |                         | S.L. absorbency, g./g. |
|--------------------|------------------------|-------------------|-------------------|---------------------|-----------------|-------------------------|------------------------|
|                    |                        | Oven              | Maximum on fabric |                     | Fibers, percent | Visual, percent/seconds |                        |
| a <sup>1</sup> --- | 30                     | 205               | 194               | C                   | 6               | 40/120                  | -----                  |
| b-----             | 10                     | 205               | 166               | C                   | 13              | 85/120                  | 0.26                   |
| c-----             | 30                     | 205               | 190               | C                   | 11              | 85/120                  | 0.32                   |
| d-----             | 30                     | 190               | 180               | D                   | 13              | 85/120                  | -----                  |
| e-----             | 30                     | 180               | 171               | D                   | 34              | 100/60                  | -----                  |
| f-----             | 30                     | 170               | 161               | D                   | 21              | 100/35                  | -----                  |
| g-----             | 30                     | 165               | 160               | D                   | 13              | 90/90                   | -----                  |

<sup>1</sup> No catalyst used.

NOTE.— Reactant solution 44.4% maleic anhydride, 1 mole NH<sub>3</sub>/mole of anhydride and 2% (based on anhydride) of sulfamic acid as a catalyst. pick-up 1.9 g./g.

I claim:

1. In the process for reacting a solution of an organic dicarboxylic acid selected from the group consisting of succinic acid, maleic acid and ortho-phthalic acid with fabric of cellulosic fibers, the improvement for providing a product dispersible in turbulent water which comprises impregnating nonwoven fabric of entangled cellulosic fibers with a solution of 1.5 to 20 times the amount of the dicarboxylic acid to be reacted with the cellulose, dissolved in water containing 1 to about 1.5 moles of ammonia per mole of acid, heating the impregnated fabric within the temperature range of 160° to 210° C. until the cellulosic fibers have a degree of substitution of about 0.15 to about 0.40, washing the fabric to remove excess reactants, and immersing the treated fabric in a buffered alkaline solution containing a deswelling salt to form the sodium salt of acid groups substituted on the cellulose.

2. A process as defined in claim 1 wherein the dicarboxylic acid is succinic acid.

3. A process as defined in claim 1 wherein the dicarboxylic acid is maleic acid.

4. A process as defined in claim 1 wherein the dicarboxylic acid is ortho-phthalic acid.

References Cited

UNITED STATES PATENTS

|    |           |        |                |       |       |
|----|-----------|--------|----------------|-------|-------|
| 25 | 2,358,387 | 9/1944 | Dreyfus        | ----- | 8—120 |
|    | 2,585,516 | 2/1952 | Thomas         | ----- | 8—120 |
|    | 2,780,228 | 2/1957 | Toney          | ----- | 8—120 |
|    | 3,526,048 | 9/1970 | Rowland et al. | ----- | 8—120 |

OTHER REFERENCES

30 St. Mard, American Dyestuff Reporter, vol. 50, No. 21, pp. 27—31 (1961).

Allen, Textile Research Journal, vol. 34, pp. 331—336 (1964).

35 Campbell et al., Textile Research Journal, vol. 35, pp. 260—270 (1965).

Rowland et al., Textile Research Journal, vol. 37, pp. 933—941 (1967).

40 GEORGE F. LESMES, Primary Examiner

J. CANNON, Assistant Examiner

U.S. Cl. X.R.

128—284; 260—224; 161—46; 8—116.2